

## UNITED STATES PATENT OFFICE.

HENRY M. SCHLEICHER, OF ROOSEVELT, AND HARVEY M. BURKEY, OF PLAINFIELD, NEW JERSEY, ASSIGNORS TO AMERICAN METAL COMPANY, LTD., OF NEW YORK, N. Y., A CORPORATION OF NEW YORK.

## PROCESS OF REFINING LEAD.

No Drawing.

Application filed March 13, 1922. Serial No. 543,471.

*To all whom it may concern:*

Be it known that we, HENRY M. SCHLEICHER and HARVEY M. BURKEY, citizens of the United States, residing at 5 Roosevelt, Middlesex County, New Jersey, and Plainfield, Union County, New Jersey, respectively, have invented certain new and useful Improvements in Processes of Refining Lead; and we do hereby declare the following to be a full, clear, and exact description of the invention, such as will enable others skilled in the art to which it appertains to make and use the same.

This invention relates to a process of refining lead, and particularly to the removal of arsenic, antimony and tin from lead and lead alloys such as lead bullion and antimonial or hard lead. The process may also be advantageously employed in the removal 20 of sulphur, selenium, tellurium and similar elements which are frequently present in crude lead.

The processes of refining lead as heretofore used are subject to certain disadvantages, particularly in the time required for the treatment and in the difficulty experienced in accomplishing the desired separation, and it is the object of the present invention to provide a simple and economical 25 process whereby impurities present in crude lead may be separated readily therefrom.

A further object of the invention is the provision of a process whereby arsenic and antimony may be separately recovered from 30 crude lead, the process thus enabling production of these elements or their compounds as by-products of the refining operation.

Another and particular object of the present invention is the improvement of a process described in our co-pending application Serial No. 512,630, filed November 3, 1921, whereby the time required to complete the 35 refining operation may be materially reduced.

Further objects and advantages of the invention will be apparent as it is better understood by reference to the following specification in which the preferred embodiments 40 of the invention are described.

In the application above referred to, we

have described in detail a process of refining lead involving the oxidation of the impurities present in the lead in the presence of a molten material having an affinity for these 55 impurities. The process involves covering a molten bath of lead with a molten layer of an alkali metal compound and introducing air under pressure to the bath to provide the oxidizing condition whereby the impurities 60 are oxidized and carried into the overlying layer. This layer may be skimmed from the surface of the bath and treated for the recovery of the metalloids.

The process described depends for its 65 success primarily upon the fact that lead, while very hot, may be blown with air without forming any appreciable amount of litharge if the metal is covered with a molten alkali metal compound and if there 70 is present in the bath of lead any element having a greater affinity for oxygen and especially any of the class of elements known as metalloids. Both of these conditions are essential because pure lead (99.95% lead) 75 will oxidize under the alkali metal compound, and, on the other hand, the presence of arsenic, antimony or other metalloids will not prevent the formation of litharge when no alkali metal compound is present. In 80 the course of our further study of the process of the prior application, we have discovered that the preferential oxidation of the contaminating elements results from the presence of small amounts of alkali metal in 85 the bath of impure lead. Thus, when the metalloids are oxidized by the passage of air through the metal, the oxide compounds of the metalloids rise to the surface and react with the molten alkali metal compounds. The presence of these small 90 amounts of alkali metal constitutes the reason for the selective oxidizing action of the air, but owing to the relatively small amounts of alkali metal thus produced, the 95 action is comparatively slow, and, as set forth in the earlier application, the successive treatments each consume approximately one hour.

We have discovered that by the addition 100 of alkali metal in a metallic condition to the lead bath, the reaction rate may be increased

materially to a point in fact which permits the successive treatments to consume only from fifteen to twenty minutes. Thus the capacity of the equipment used may be multiplied from three to four times with corresponding saving in the cost of the refining operation.

As stated, an alkali metal such as metallic sodium may be added directly to the lead bath while the latter is covered by a layer of an alkali metal compound, and, upon the introduction of the blast of air, selective oxidation will occur rapidly with the result that the antimony and other metalloids present will be oxidized and carried into the overlying alkali metal compound layer. The alkali metal in the bath apparently acts as a catalyst since it remains therein until substantially all of the metalloids have been eliminated. The alkali metal is then also eliminated, probably combining with the small amount of litharge which is formed at the end of the treatment, and which serves by its appearance as an indication that the reaction is completed. The lead bath, after the completion of the treatment, is free from alkali metal.

It is preferable, however, to employ the alkali metal in the form of an alloy. Thus a sodium lead alloy may be utilized. A sodium antimony alloy is also suitable for use, and in the further treatment the antimony may be recovered for further use. One advantageous method of thus recovering the antimony is to leach the slag for the purpose of recovering the excess of alkali metal compound. The antimony compound is insoluble and is readily separated. By heating this compound with a proportion, e. g., 15% of charcoal, a metallic mass is obtained which consists essentially of antimony with 15 to 20% of metallic sodium. The metallic mass may be introduced into the bath of molten lead with very satisfactory results.

As a specific example of the application of the invention, we have found that by adding an alloy of lead or antimony containing 15 to 20% of metallic sodium to the bath of molten lead in an amount equal to approximately five tenths of 1% of the weight of the metal bath and then subjecting the bath to the blast of air, the desired separation of metalloids may be accomplished in from fifteen to twenty minutes, that is to say, the proportion of the metalloids which may be removed in a single treatment may be oxidized and carried into the overlying layer of alkali metal compound in the time mentioned. In practical operations, it is sufficient that a proportion of caustic soda or other suitable alkali amounting to 2.5% of the weight of the metal bath be disposed as a layer thereon and that an alkali metal in a free condition or combined

as an alloy with lead or antimony, for example, be added to the bath in such proportion that the alkali metal shall amount to approximately one-tenth of 1% of the weight of the bath.

It is not necessary to add alkali metal each time a layer of caustic alkali is added. One such addition may suffice for the entire operation. The air is not introduced into the bath during skimming or while adding a new lot of caustic alkali.

It is to be understood that after each period of blowing when the layer of alkali metal compound has begun to stiffen, it is removed and the operation is repeated until substantially all of the metalloids have been separated.

The process is preferably carried out in a suitable iron or steel pot or converter which is heated by a furnace to a temperature of from 625 to 700° C. The converter is provided with tuyères through which the air, which is preferably pre-heated, is introduced to the lead bath. The tuyères may extend into the bath for some distance to insure the proper dissemination of the air therein.

The skimmings from the lead bath, consisting of the alkali metal compound with oxidized metalloids combined therewith, are thrown into water with the resulting production of a strong caustic solution and an insoluble residue. The solution is decanted and the residue is dried and treated for the recovery of antimony or antimony compounds, or as hereinbefore set forth, a proportion of the antimony compounds may be reduced to provide the antimony sodium alloy for the further treatment of the lead bath. The residue contains substantially 60% of antimony mostly in pentavalent state, about 18% of sodium oxide, and small amounts of iron and lead. Any lead shot carried over in the caustic soda may be separated from the antimony residue and returned to the lead bath. The solution is subjected to a suitable precipitating agent to throw out the arsenic which may be worked up to produce arsenic or arsenic compounds. The solution is then evaporated preferably by fine gases from the melting furnace, and when concentrated and fused, the caustic soda may be reused.

If the lead bullion contains arsenic and antimony, the greater part of the arsenic is eliminated in the early part of the process, that is to say, in the first skimmings of caustic soda. Substantially all of the arsenic is soluble so that it is almost completely separated from the antimony.

If tin be present it is also soluble and may be recovered by suitable treatment.

Any silver which may be present in the lead remains therewith since it is unaffected by the process and does not enter the skimmings. The silver may be separated from

the lead after the completion of the process in accordance with the usual practice.

From the foregoing, it will be understood that the process herein described provides for the effective separation of impurities from lead in a simple and economical manner, and particularly in a more rapid manner than is possible under the practice described in the earlier application. Soft lead may be produced from lead containing considerable quantities of arsenic and antimony with a minimum of expense.

Various changes may be made in the details of the process within the scope of the accompanying claims and without departing from the invention or sacrificing any of the advantages thereof.

We claim:

1. A method of refining lead, which comprises subjecting the molten lead to an oxidizing condition in the presence of a molten material capable of combining with oxides of the impurities present in the lead, accelerating the reaction by the addition of an alkali metal to the molten lead, and separating the molten material with the impurities from the lead.

2. A method of refining lead, which comprises subjecting the molten lead to an oxidizing condition in the presence of a molten material capable of combining with oxides of the impurities present in the lead, accelerating the reaction by the addition of an alloy containing an alkali metal to the molten lead, and separating the molten material with the impurities from the lead.

3. A method of refining lead, which comprises subjecting the molten lead to an oxidizing condition in the presence of a molten material capable of combining with oxides of the impurities present in the lead, accelerating the reaction by the addition of an alloy of lead with an alkali metal to the molten lead, and separating the molten material with the impurities from the lead.

4. A method of refining lead, which comprises subjecting the molten lead to a current of an oxidizing gas in the presence of a molten material capable of combining with oxides of the impurities present in the lead, accelerating the reaction by the addition of an alkali metal to the molten lead, and separating the molten material with the impurities from the lead.

5. A method of refining lead, which comprises subjecting the molten lead to an oxidizing condition in the presence of a molten alkali metal compound and of an alkali metal, and separating the alkali metal compound with the impurities from the lead.

6. A method of refining lead, which comprises subjecting the molten lead to a current of an oxidizing gas in the presence of a molten alkali metal compound and

of an alkali metal, and separating the alkali metal compound with the impurities from the lead.

7. A method of refining lead, which comprises forcing a current of air through the molten lead in the presence of a molten material capable of combining with oxides of the impurities present in the lead, accelerating the reaction by the addition of an alkali metal to the molten lead, and separating the molten material with the impurities from the lead.

8. A method of refining lead, which comprises forcing a current of air through the molten lead in the presence of a molten alkali metal compound and of an alkali metal, and separating the alkali metal compound with the impurities from the lead.

9. A method of refining lead to remove antimony therefrom, which comprises forcing a current of air through the molten lead in the presence of an alkali metal hydroxide and of an alkali metal, and separating the alkali metal compound containing antimony from the lead.

10. A method of refining lead to remove antimony therefrom, which comprises subjecting the molten lead to an oxidizing condition in the presence of a molten alkali metal compound and of an alloy containing antimony and an alkali metal, and separating the alkali metal compound containing antimony from the lead.

11. A method of refining lead to remove antimony therefrom, which comprises subjecting the molten lead to an oxidizing condition in the presence of a molten alkali metal compound and of an alloy containing antimony and an alkali metal, separating the alkali metal compound containing antimony from the lead, leaching the alkali metal compound to recover insoluble antimony compounds therefrom, and reducing the antimony compounds to provide the alloy of antimony with an alkali metal.

12. A method of refining lead to remove impurities therefrom, which comprises covering the molten lead with a molten layer of a material capable of combining with oxides of the impurities present in the lead, adding an alkali metal to the molten lead, forcing an oxidizing gas through the mass, and separating the molten material with the impurities from the lead.

13. A method of refining lead to remove impurities therefrom, which comprises covering the molten lead with a molten layer of an alkali metal compound, adding an alkali metal to the molten lead, forcing an oxidizing gas through the mass, and separating the alkali metal compound from the lead.

14. A method of refining lead to remove impurities therefrom, which comprises covering the molten lead with a layer of molten material having a selective affinity for the

impurities present in the lead, adding an alloy containing an alkali metal to the molten lead, forcing an oxidizing gas through the mass, and separating the molten material with the impurities from the lead.

15. A method of refining lead, which comprises covering the molten lead with a layer of molten material capable of combining with oxides of the impurities present in the lead, adding an alloy containing lead and an alkali metal to the molten lead, forcing an oxidizing gas through the mass, and separating the molten material with the impurities from the lead.

16. A method of refining lead to remove impurities therefrom, which comprises covering the molten lead with a molten layer of an alkali metal compound, adding an alloy containing an alkali metal to the molten lead, forcing an oxidizing gas through the mass, and separating the alkali metal compound from the lead.

17. A method of refining lead to remove impurities therefrom, which comprises covering the molten lead with a molten layer of an alkali metal compound, adding an alkali metal to the molten lead, forcing an oxidizing gas through the mass, skimming the alkali metal compound from the lead, and repeating the operation with further quantities of alkali metal compound and alkali metal until the impurities are substantially exhausted.

18. A method of refining lead to remove impurities therefrom, which comprises covering the molten lead with a molten layer

of an alkali metal compound, adding an alkali metal to the molten lead, forcing an oxidizing gas through the mass, skimming the alkali metal compound from the lead, repeating the operation with further quantities of alkali metal compound and alkali metal until the impurities are substantially exhausted, leaching the skimmings to separate insoluble material from the alkali metal compound, evaporating the solution and returning the recovered alkali metal compound for further use.

19. A method of refining lead to remove impurities therefrom, which comprises subjecting the impurities in the molten lead to selective oxidation in the presence of an alkali metal.

20. A method of refining lead to remove impurities therefrom, which comprises subjecting the impurities in the molten lead to selective oxidation in the presence of an alkali metal added to the lead in the form of an alloy.

21. A method of refining lead, which comprises subjecting the molten lead to an oxidizing condition in the presence of an alkali metal.

22. A method of refining lead, which comprises subjecting the molten lead to an oxidizing condition in the presence of an alkali metal and in the presence of a molten alkali metal compound.

In testimony whereof we affix our signatures.

HENRY M. SCHLEICHER.  
HARVEY M. BURKEY.